

G. M. WILLIS.

## PROCESS FOR THE TREATMENT OF ORES AND MINERALS.

APPLICATION FILED JAN. 21, 1915.

1,313,970,

Patented Aug. 26, 1919.



Witnesses. 35

F. J. Horner  
James L. Fidler.

Inventor:  
George M. Willis  
By Bell & Howley

# UNITED STATES PATENT OFFICE.

GEORGE M. WILLIS, OF CHICAGO, ILLINOIS.

## PROCESS FOR THE TREATMENT OF ORES AND MINERALS.

1,313,970.

Specification of Letters Patent. Patented Aug. 26, 1919.

Application filed January 21, 1915. Serial No. 3,429.

*To all whom it may concern:*

Be it known that I, GEORGE M. WILLIS, a citizen of the United States, residing at Chicago, in the county of Cook and State 5 of Illinois, have invented certain new and useful Improvements in Processes for the Treatment of Ores and Minerals, of which the following is a specification.

My invention relates to an improved process for the treatment of ores and minerals 10 by which foreign substances are removed from them or so changed in form by treatment with electric current or gases or both that the metal contained in the ores or 15 minerals may subsequently be recovered by suitable processes in purer form and more efficiently than has been possible by processes used heretofore. By my process I subject the ores or minerals to the flow of 20 current of suitable strength at a temperature insufficient to fuse the same and at the same time supply to the mass of the ore or mineral highly superheated steam and compressed air, which, preferably, are applied 25 alternately to the ore or mineral being treated. If desired, the superheated steam may be used without the compressed air, although under such conditions the results secured are not as efficient.

While I find that the treatment referred 30 to above produces a marked effect upon the ore or mineral treated, I am not aware of the exact nature of the change produced in the ore or mineral, excepting that substances which are contained in the ore or 35 mineral, such as sulfur, phosphorus, etc., are either wholly or partially driven off or so changed as to their molecular arrangement as to be more readily removable in 40 the subsequent treatment so as to leave the final product free from these substances, which, if they remained therein, would seriously modify the quality of the metal recovered from the ore or mineral. I also 45 find that by my process minerals which are naturally very refractory are modified as to their characteristics; as, for example, in the case of refractory minerals containing gold the yield of gold after treatment is 50 much higher than where the mineral is subjected to the same processes of recovery without being treated by my process.

The several drawings illustrating my invention are as follows:

Figure 1 shows in plan view a furnace

for treating the ores and minerals, and also shows diagrammatically the apparatus and circuit connections employed in connection with said furnace;

Fig. 2 is a vertical sectional view through 60 the furnace shown in Fig. 1;

Fig. 3 is a view taken from the left-hand 65 of the left-hand electrode support contained in the furnace shown in Figs. 1 and 2; and

Fig. 4 is a sectional view through the 70 electrodes showing the supports used at the right-hand ends of the same, said view being taken along the line 4-4 of Fig. 2.

Similar numerals refer to similar parts 70 throughout the several views.

As shown in Figs. 1 and 2, the furnace 75 consists preferably of a metallic casing 10 lined with heat-resistant material 11, which material extends on the four sides of the furnace, and across its bottom, a removable cover 12 of similar construction being provided to close the furnace when in operation. The heat-resistant material 11 is preferably made of porous fire clay which may 80 be formed by mixing granulated cork or similar substance with the fire clay before making the lining thereof, as a result of which when the furnace is heated the cork, or similar material, is burned out, leaving 85 air cells throughout the hardened fire clay. Other fire-resistant materials may, of course, be employed instead of the fire clay if desired. In constructing the lining of the furnace it is not necessary that the heat-resistant 90 material shall be very highly refractory, for the reason that the temperatures employed in the furnace are not excessive. The heat-resisting lining serves rather as a heat-insulator for the purpose of preventing loss 95 of the heat developed in the furnace.

A gas delivering device 13 is placed upon the bottom of the furnace and provided with a supply pipe 14 extending to a superheating coil 15, the other end of which, as indicated in Fig. 1, is connected with a pressure-controlling valve 16 from which a pipe 17 extends to a two-way cock 18 by which connection may be established as desired, either with a boiler 19 through the pipe 20, 100 or through the pipe 21 with a tank 22 containing compressed air. The boiler 19 may be heated by any suitable means, a gas burner 23 being shown in Fig. 1 for accomplishing this result. The supply of gas 105 110

to the burner 23 may be controlled as desired by a valve 24 located in the pipe connected with said burner. The superheating coil 15 is preferably inclosed in a casing 25 5 to fully utilize the heat from a gas burner 26 located in the lower portion of said casing, and the supply of gas to said burner 26 may be controlled as desired by a valve 27 located in the pipe connected with the 10 burner. Suitable apertures may be provided in the casing 25, as indicated, to permit proper burning of the gas, and the cover 28 of the casing is preferably removable to permit the assembling of the super- 15 heating mechanism.

The gas delivering mechanism 13 is of a construction similar to that employed in gas burners so that the gases delivered by such mechanism to the furnace are widely and 20 evenly distributed through the material in the furnace, and to prevent the material entering the device 13 a screen 28 is placed above the said device and extends entirely across the lower portion of the furnace, in 25 which position it is supported in any suitable manner by blocks 29 of heat-resistant material. The furnace also contains a plurality of electrodes or current terminals constructed and related as follows: At the left- 30 hand side of the furnace, as shown in Figs. 1 and 2, a plate 30 is disposed, which plate is preferably of iron or steel, and has rigidly secured in it one end of each of the electrodes or terminals 31, the other ends of 35 which are supported by a grid 32 of the general conformation indicated in Fig. 4. A second set of electrodes or terminals 33 is disposed between and alternating with the electrodes or terminals 31, the right-hand 40 ends of these electrodes 33 being secured in a plate 34 located at the right-hand side of the furnace, which plate is similar to the plate 30, and these electrodes or terminals 33 extend through the clearance openings 45 provided in the grid 32, and have their left-hand ends supported by a second grid 35 similar to the grid 32, to provide clearance openings around the electrodes or terminals 31. The grids 32 and 35 are constructed 50 preferably of iron or steel, and to facilitate assembling the electrodes it is preferable that they should be readily removable from the electrodes if desired, and that when in supporting position in engagement with the 55 electrodes they may be held in such position by means of set screws 36, as indicated for the grid 32 in Fig. 4. The material of which the electrodes or terminals is constructed is immaterial as long as it is a sufficiently good conductor of electricity to 60 supply electric current to the material to be treated in the furnace. Thus, for example, either carbon or metal may be employed, and in carrying out my process in practice I 65 find it desirable to construct these electrodes

of mild steel or iron, since this material is a sufficiently good conductor of electricity for this purpose, and the temperatures employed are not sufficiently high to melt or disintegrate the iron or steel. Furthermore, 70 the electrode construction may be cheaply and effectively made by making the electrodes of iron or steel. In this manner the electrode construction may be made sufficiently strong so that there is no danger of 75 breakage of the electrodes or the parts connected therewith by placing the ore or mineral in the furnace and removing the same from the furnace.

To supply the alternating current to the 80 furnace the plate 30 is connected by a wire 37 with one terminal of the secondary winding 38 of an alternating current transformer, the other terminal of which winding is connected by wire 39 with the pivotal point of 85 a rheostat switch 40, one terminal of the resistance 41 of said rheostat being connected by wire 42 with the other plate 34 located in the furnace. The primary winding 43 of the transformer has its terminals connected, 90 as indicated, with a source of alternating current supply 44, which may consist of alternating current feed wires used for distribution purposes in cities and towns, or an alternating current generator where such 95 distributing feed wires are not available.

In carrying out my process the ore or mineral is first broken up into a sufficiently divided condition to freely enter between the electrodes 31 and 33, in which condition it is 100 dumped into the furnace on the screen 28 and in sufficient quantity to practically fill the furnace. The cover of the furnace is then put in place, and by means of the switch 40 alternating current is supplied to the 105 electrodes 31 and 33 at a voltage sufficient to cause such an amount of current flow through the ore or mineral as will heat the same after a short time to a cherry red heat. As the temperature of the ore or mineral is 110 increased, the amount of voltage impressed upon the electrodes is decreased from time to time so that when the contents of the furnace have been heated to the required temperature, which, as referred to, is preferably 115 not above a cherry red heat, but a small quantity of current flow is required to maintain the heated ore or mineral at that temperature. When substantially the degree of heat of the ore or mineral referred to has 120 been reached, the cock 18 is operated to admit steam from the boiler 19 through the superheating coil 15 to the device 13, the boiler 19 and the superheating coil 15 having previously been placed in operation so as 125 to supply superheated steam when the cock is thus operated. The valve 16 is adjusted so that the pressure of the steam delivered to the device 13 is sufficient to force the superheated steam from the device 13 into the ore 130

or mineral but insufficient to blow the particles of ore or mineral from the furnace.

In practice I find that the pressure required at the device 13 is very low, being not over a fraction of a pound to the square inch, so that there is no need to clamp the cover of the furnace in place to prevent its being lifted by the pressure in the furnace. In practice it is preferable that the cover 10 of the furnace shall fit somewhat loosely upon the furnace so that the gases introduced into the furnace and the gases resulting from the treatment of the ore or mineral may readily escape from the furnace without, however, permitting the escape of an undue amount of heat. The super-heating coil 15, which is preferably of brass or copper, although it may be made of other metal if desired, should at all times be heated sufficiently 20 so that the steam delivered through the pipe 14 to the device 13 is heated sufficiently hot so that the dry steam produced is dissociated and broken up into its constituent gases, to-wit, hydrogen and oxygen, which gases are delivered to and from the device 13 in this liberated and highly heated condition. This condition of heating of the pipe 15 is attained when the latter is heated to a bright red heat. 30 After the dissociated steam has been passed through the furnace for a short time, as, for example, from ten to twenty minutes, the cock 18 is moved to a position interrupting the flow of steam from the pipe 20 to the pipe 17 and establishing communication between the pipes 21 and 17, for which condition air is supplied from the tank 22 through the heating coil 15 and delivered to the device 13, and thus to the ore or mineral 40 in the furnace. The interval of this treatment is preferably somewhat shorter than the treatment with the dissociated steam, and then the cock 18 is again moved to its position, interrupting communication between the pipes 21 and 17 and establishing communication between the pipe 17 and the boiler 19, and the alternate treatment of the ore or mineral in the furnace with the dissociated steam and ore is continued for a sufficient length of time to remove from the ore or mineral to the desired degree the substances which are attacked by the highly heated gases delivered to the furnace. In practice I find that a treatment of iron ore 55 for a period of three quarters of an hour to an hour will, so far as I am able to determine by analysis, serve to completely remove from the recovered metal all of the sulfur, phosphorus and impurities contained in the ore originally, although the ore is practically unchanged physically by its treatment in the furnace.

It will be understood that while I have shown the air tank diagrammatically, this tank in practice will be of a sufficient ca-

pacity and provided with suitable charging apparatus in the way of compressors well known in the art to maintain at all times a sufficient quantity of compressed air in the tank at a proper pressure for delivery to the gas delivering mechanism 13, and that preferably the pressure in the tank should be substantially the same as the pressure generated in the steam boiler, so that the valve 16 may be set in the proper position for any particular material being treated, and remain in that position as long as the same kind of material is under treatment, assuming that the pressures in the boiler and air tank remain substantially constant. 80

The principal change that is produced in the physical appearance of the ore by the treatment referred to is that the ore is given a finely-powdered condition and is somewhat discolored by the heating, and, possibly, by the action of the gases, but as far as the chemical condition of the ore is concerned the only change produced is the driving off of the sulfur, and other substances, without, however, changing the condition of the metallic portion of the ore. For example, in treating iron ore, at the end of the treatment the ore is still iron oxid, and no metallic iron is produced, for the reason that the temperatures employed 90 are insufficient to produce any reducing effect.

The temperature to which the ore or mineral is heated varies somewhat with different ores, depending upon the reducing 100 temperature of said ores, it being an important consideration in carrying out my process that the temperature shall not reach the reducing temperature of the ore or mineral. For practical purposes an indication of the proper temperature is had when the ore or mineral is heated to redness, which is attained by heating the ore or mineral to from 1200 degrees to 1500 degrees Fahrenheit. 110

The ore thus treated is then subjected to a smelting operation of any desired and well known kind for the purpose of reducing the ore to metallic form, as, for example, by fluxing the ore by means of suitable heat with carbonate of soda, borax, and charcoal, although other fluxes may be employed if desired and other smelting operations employed, depending upon the results desired and the ore being treated. 115

In the case of iron ore treated as described above, I find that upon subsequently smelting the treated ore in the manner referred to, I secure a quality of iron having radically different physical and chemical characteristics from iron produced by any other process of which I am aware. The resulting iron is, as far as I am able to determine by analysis, chemically pure and extremely ductile and malleable, and, furthermore, of 125 130

very different magnetic properties than iron usually has, for I find upon test that the iron thus produced is not highly magnetic.

My process and apparatus are not applicable alone to iron ores, since other ores may be similarly treated when it is desired to free the ores from the presence of substances that may be attacked by the gases delivered to the furnace and driven off in volatilized or oxidized condition. Thus, for example, I find that refractory gold-bearing ore when treated in my furnace as described above is, in some manner unknown to me, changed, so that the gold contained in said ore is available and may be recovered to a much greater degree than is possible without so treating the ore. Certain tests that I have made in this connection have shown a recovery of gold from such refractory ore double in amount to that which could be recovered without first so treating the ore.

While my process is particularly adapted to iron ores of various kinds and ores or minerals bearing and containing precious metals, it will be understood that it is equally applicable to any ore or mineral having a composition such that it will not be undesirably changed or transformed by the temperature of the treatment in the furnace and from which ore or mineral it is desired to remove substances or impurities which may be volatilized, oxidized, or changed in physical or chemical form by the gases delivered to the furnace in connection with the action of the electric current flowing through the furnace. My process and apparatus are further applicable to the partial elimination of impurities by continuing the treatment for only a portion of the time required for the complete elimination of said substances, so that as is desirable in some cases a resulting metal may be produced in which the sulfur content, for example, shall not exceed a specified percentage, the advantage of the partial removal of the sulfur in such cases being that the expense of the treatment is reduced.

It will be understood that it is not necessary in all cases to use the alternating current in carrying out my process, as the impurities may be removed with a fair degree of success under certain conditions by heating the material to be treated in any desired manner; as, for example, by the application of external heat to the furnace, or in any equivalent way, and subjecting the material to the action of the dissociated steam. This way of carrying out my process may be used, for example, in case it is desired to remove but a part of the substances which may be volatilized, oxidized or changed, and where it is desired to more completely remove these substances, better results may be secured by alternately treating the material with the dissociated steam and heated air, although still

maintaining the temperature of the material by the application of heat in some other way than by the electric current. Where complete and effective elimination of said substances is desired, however, this can be most effectively accomplished by maintaining the temperature of the material at the desired point by means of the alternating current flow, as described above, and at the same time alternately treating the material with dissociated steam and heated air.

While I have pointed out above that the temperature during the treating of the ore or mineral to eliminate the undesirable substances is to be maintained below the fusing temperature of the ore or mineral, it is to be understood that in certain cases where it is desired to secure but a partial elimination of these undesirable substances, which may be driven off, as above described, this result may be secured by subjecting the ore or mineral to the action of the electric current or heated gases, or both, during the heating of the same, where the result of the continued heating is to fuse or melt the ore or mineral, the portion of the heating operation prior to the fusion or melting being of sufficient duration to effect the desired amount of elimination before the fusion or melting occurs.

It will also be understood that while the best results are secured by the use of alternating current, other forms of electric current may be employed in carrying out my process, particularly where the heating action of the current is depended upon to heat the ore or mineral to the proper temperature or to maintain said heated condition.

One of the marked advantages which may be secured by the treatment of iron ore having a large phosphorus content so as to eliminate a part of said phosphorus is that sufficient of said phosphorus is eliminated by such treatment as to permit of subsequent manufacture of steel by the Bessemer process for the production of steel rails, etc., having a phosphorus content below a specified limiting maximum amount. It will readily be appreciated that one of the marked advantages of treating iron ore by my process so that all of the substances which may be removed by volatilizing, vaporizing and changing the same is that the resulting pure iron is available for subsequent treatment by any of the processes well known in the art for the production of high-grade steels having any desired chemical composition to meet the varying requirements of the art for such steels.

It will be understood that the electric current may be supplied to the material in the furnace by any desired arrangement of electrodes as long as the electrodes are in such relation to the contents of the furnace that the current used will flow through the

furnace and the material contained therein, either for the purpose of heating the material contained in the furnace or assisting in the purifying action characterizing my process, or both, as desired. It will also be understood that I may treat the ores or minerals either with hydrogen or oxygen or both whether said gases are produced by the dissociation of steam or otherwise.

5 10 I therefore consider my invention to include broadly the process of treating ores and minerals by electric current or highly heated gases, or both, as described above, and any form of apparatus that will carry 15 out this process substantially along the line indicated broadly above.

What I claim is:

1. The process of treating ores and minerals, which consists in subjecting them to 20 the action of alternating current flow and alternately passing through the ore or mineral the gases of dissociated steam and air.

2. The process of treating ores and minerals, which consists in subjecting them to 25 the action of alternating current flow and the alternate action of the gases of dissociated steam and highly heated air.

3. The process of treating ores and minerals, which consists in treating them without 30 fusion of the ore or mineral with alternating current flowing through them and alternately with the gases of dissociated steam and air.

4. The process of treating ores and minerals, which consists in producing an alternating current flow between a plurality of alternating electrodes in the mass of the ore or mineral, and alternately supplying 35 to the ore or mineral the gases of dissociated steam and air.

5. The process of treating ores and minerals, which consists in producing an alternating current flow between a plurality of alternating electrodes in the mass of the ore or mineral without fusion of the ore or min- 40

eral, and alternately supplying to the ore or mineral the gases of dissociated steam and air.

6. The process of treating ores and minerals, which consists in subjecting them to 50 the flow of alternating current, and alternately supplying to them the gases of dissociated steam immediately after the dissociation of the same, and highly heated air.

7. The process of treating ores and minerals, consisting in subjecting them to the 55 flow of alternating current through a plurality of paths from electrodes alternately disposed throughout the ore or mineral, and alternately subjecting the ore or mineral to 60 the action of the gases of dissociated steam immediately after the dissociation of the same, and highly heated air.

8. The process of treating ores, minerals, and similar materials, consisting in heating 65 them to a temperature below their reducing temperature, and subjecting them alternately to the action of the gases of dissociated steam and air.

9. The process of treating ores, minerals, and similar materials, consisting in heating 70 them to a temperature below their reducing temperature, and subjecting them alternately to the action of the gases of dissociated steam immediately after the dissociation 75 of the same and the action of heated air.

10. The process of treating ores and minerals, consisting in subjecting them to the action of electric current flow, and passing 80 through the ore or mineral the gases of dissociated steam and air.

In witness whereof, I hereunto subscribe my name this 12th day of January, A. D. 1915.

GEORGE M. WILLIS.

Witnesses:

ALBERT C. BELL,  
L. E. HANNEN.

Copies of this patent may be obtained for five cents each, by addressing the "Commissioner of Patents,  
Washington, D. C."